

Oct. 11, 1927.

1,644,746

K. H. W. RAMSAY

DRY CELL ELECTRODE AND METHOD OF MAKING THE SAME

Filed Dec. 26, 1925



INVENTOR  
Karl Henrik William Ramsay  
BY  
*Frederick Brutenberg*  
his ATTORNEY

## UNITED STATES PATENT OFFICE.

KARL HENRIK WILLIAM RAMSAY, OF SUMMIT, NEW JERSEY, ASSIGNOR TO DIAMOND ELECTRIC SPECIALTIES CORP. OF NEWARK, NEW JERSEY, A CORPORATION OF NEW JERSEY.

## DRY-CELL ELECTRODE AND METHOD OF MAKING THE SAME.

Application filed December 26, 1925. Serial No. 77,680.

My present invention relates generally to dry cells and has particular reference to the type which embodies a bobbin comprising a carbon rod electrode carrying a molded mix.

5 Cells of this character generally comprise a second electrode consisting of a zinc cup in which an electrolyte is carried, and it has been found necessary to provide means for binding the bobbin together by an enclosing envelope so as to prevent disintegration thereof when it is initially assembled with the zinc cup electrode by dipping it into the electrolyte.

Means have been provided comprising 15 bags of cheese-cloth or similar fabric which are generally tied about the bobbin by manual labor. Bags of this type have the essential property of being permeable to the electrolyte, but their utilization entails much 20 additional expense and time due to the operation required to tie them in place.

Where I have attempted to enclose the bobbins in coatings of plaster of Paris or similar material instead of in fabric bags, I 25 have found that numerous disadvantages are entailed, including the comparatively long period required for the plaster to set, and the necessity for preparing the plaster in comparatively small batches to minimize 30 as far as possible, the waste which occurs even under favorable conditions due to the nature of the plaster in starting to set as soon as it is moistened and in being incapable of resoftening after it has set.

35 Moreover, the comparatively lengthy association of the bobbin with a moist material may have a detrimental effect upon the firmness of the bobbin; and the moisture increases the possibility of the very disintegration which it is desired to guard against.

It is an object of the present invention to provide a coating whose application constitutes an extremely simple operation, entailing an almost negligible amount of time, 45 and producing a dry protective film almost instantaneously; the film being not only permeable to electrolytic flow but sufficiently tough and strong to fulfill its binding purpose.

50 Another object of the invention is to provide a bobbin-coating method wherein waste of material is entirely prevented, the particular material in contemplation being of a

character which permits preparation in large quantities without impairing its utility over a period of time, due to the fact that its hardening or thickening may be controlled.

A further object is to provide a method of coating during which the bobbin may be retained in its driest possible condition, thereby increasing the output efficiency by preventing wastage of bobbins by disintegration.

My invention contemplates the use of a soluble material whose hardening is due to the rapid evaporation of the solvent rather than the combination of the latter with the base, as in the case of plaster of Paris. The use of such a coating makes it possible to 70 prepare large quantities thereof, and to utilize it as desired, without regard to lapse of time. Furthermore, a coating of this nature permits the time and rapidity of drying to be controlled by the character of solvent 75 used. My invention also contemplates the addition to the coating material of various salts which are soluble in the electrolyte and which enhance the subsequent permeability 80 of the dried coating.

Among the materials having not only the essential properties required for a utilization of this character, but also the desirable characteristics hereinbefore referred to, I have found that varnishes, such as lacquers, 85 various gums, and cellulose derivatives, are very satisfactory; and one embodiment of my invention contemplates the utilization of materials of this character.

In a preferred embodiment, I coat the 90 bobbins with a varnish, and thereupon permit the usual solvent to evaporate. I prefer to use solvents which are capable of very rapid evaporation, such as the organic solvents illustratively exemplified by alcohol, 95 whereby the dried film or membrane may be produced in as short a time as five seconds.

Although the use of any particular varnish or solvent is optional, depending upon the rapidity of drying and the nature of the 100 coating desired, I have found it preferable to utilize a cellulose derivative such as pyroxylin dissolved in any of its well-known solvents, such as alcohol-ether, amyl acetate, wood alcohol, etc. I have found that collodion lacquer, commonly known as collodion, 105

is particularly suitable and well adapted for the contemplated purpose; and in a preferred method of carrying out the invention, the collodion is pre-treated by the addition 5 of zinc chloride or other suitable salt which is soluble in the electrolyte to be used, although such pre-treatment is optional.

For the attainment of the foregoing objects and such other objects as may herein- 10 after appear or be pointed out, I have illustrated one form of dry cell, constructed in accordance with my invention, in the accompanying drawing, which represents in eleva- 15 tional cross-section an assembled and complete dry cell.

A carbon rod 10 is utilized as a base for the usual mix 11 which is applied thereto by tamping or otherwise to constitute the bobbin. The mix 11 may comprise the usual 20 carbon granules mixed with manganese dioxide and preferably a small amount of zinc chloride or other suitable binding agent. Before the bobbin is inserted into the electrolyte 12 which is carried within the zinc 25 cup 13, it is coated, preferably by dipping, with a material dissolved in a solvent capable of rapid evaporation; in a preferred embodiment, with a thin film or membrane of varnish 14. The bobbin is dipped sufficiently, 30 or similarly coated, to enclose the entire bobbin, including the top and bottom thereof and a small portion of the projecting rod 10.

The electrolyte 12 may comprise a solution of zinc chloride and sal ammoniac mixed 35 with flour and starch in a well-known manner to provide a pasty mass which will subsequently gelatinize. Sufficient electrolyte is placed into the zinc cup to completely encircle the bobbin 11 after the latter has been 40 inserted into the cup into a position resting upon a suitable insulating washer 15 covering the base 13. Thereupon a second washer 16 is inserted to provide an air space 17 be- 45 tween itself and the level of the electrolyte 12. A cap 18 is then applied to the top of the rod 10, and a suitable sealing substance 19, such as sealing wax, is applied above the washer 16 to seal the battery, leaving only the end portion of the cap 18 exposed.

It will be understood that permeability to 50 electrolytic flow is an essential characteristic of the coating 14. The permeability may be increased when desired by the addition of suitable salts soluble in the electrolyte, or by 55 permitting coated bobbins to dry in an atmosphere of moist air. I prefer to prepare the coating by mixing commercial collodion (U. S. P.) in equal amounts with a saturated alcoholic solution of zinc chloride.

Although it is optional whether the bob- 60 bin is coated by spraying, direct application, or dipping, or by any other method, I prefer to apply the coating by dipping, for the reasons that absolutely no waste is entailed, 65 large quantities of the bobbins may be coated

at one time, and the extent of the coating upon the carbon rod itself may be carefully and accurately controlled.

Because of the nature of the solvent, a dry and tough final coating will be produced 70 within approximately five seconds after the bobbins have been dipped. This constitutes a very important advantage in the manufacture of cells, because no time need be wasted between the dipping operation and the operation wherein the bobbins are inserted into the electrolyte. Moreover, absolutely no waste is entailed because the coating may be prepared in very large quantities since the effects which standing may have upon the 75 coating material may be easily remedied by the mere addition of a small amount of extra solvent. Where varnish is used, the nature of the varnish permits extremely thin coat- 80 ings to be produced having thicknesses in 85 the nature of approximately .005 of an inch. Films of this thickness are however suffi- 85 ciently tough and strong to form efficient protective coatings, and this extreme thin- 90 ness combined with the absence of waste of material, permits many more bobbins to be coated with a given amount of material than has been possible heretofore. Furthermore, 95 extreme thinness, combined with strength, is extremely desirable in constructions of this 95 character for the further reason that exces- 95 sive resistance to electric current is effectu- ally prevented.

It will thus be seen that I have provided a method of coating which is extremely effi- 100 cient not only from the standpoint of strength and permeability of the membrane produced, but also from the standpoint of economy, a great saving being effected not only by the elimination of waste but by the 105 reduction of labor required, time expended, and material used.

It will be obvious that various changes may be made in the details herein described for the purpose of explaining the nature of 110 my invention without departing from the spirit and scope of the invention as expressed in the appended claims.

I claim:-

1. A dry cell bobbin having a surface 115 coating of an inherently permeable varnish forming an integral part thereof.

2. A dry cell bobbin having a surface coating of varnish mixed with a substance soluble in the electrolyte of the cell. 120

3. A dry cell bobbin having an inherently permeable surface coating consisting essen- 125 tially of pyroxylin.

4. A dry cell bobbin having a coating of varnish mixed with zinc chloride. 125

5. The method of preparing a dry cell bobbin which comprises molding a material into electrode form susceptible of disintegra- 130 tion, coating said form with a rapidly dry- ing varnish which on drying deposits a

coherent supporting surface film permeable to electrolytic flow, and causing the same to dry.

6. The method of preparing a dry cell bobbin which comprises forming an electrode body which is susceptible of disintegration, coating said body with a rapidly drying collodion solution which on drying deposits a coherent supporting film permeable to electrolytic flow, and causing the same to dry.

7. The method of preparing a dry cell bobbin which comprises molding a material into electrode form susceptible of disintegration, coating said form with a rapidly drying varnish containing a substance soluble in the electrolyte of the cell and which on

drying deposits a coherent supporting film permeable to electrolytic flow, and causing the same to dry. 20

8. The method of preparing a dry cell bobbin which comprises forming an electrode body which is susceptible of disintegration, coating said body with a rapidly drying collodion solution containing a substance 25 soluble in the electrolyte of the cell which on drying deposits a coherent supporting film permeable to electrolytic flow, and causing the same to dry.

In witness whereof, I have signed and 30 sealed this specification this 24th day of November, 1925.

KARL HENRIK WILLIAM RAMSAY.